# EUROPEAN PATENT APPLICATION

(11) **EP 0 538 820 A1**
(43) Date of publication of application: **28.04.1993**
(21) Application number: 92117999.0
(22) Date of filing: 21.10.1992
(51) Int. Cl.: G03C 5/26

(54) **Method of wrapping photographic treating agents**

(30) Priority: 21.10.1991 JP 301005/91
(71) Applicant: FUJI PHOTO FILM CO., LTD., Kanagawa (JP)
(72) Inventor: Hori, Satoshi, c/o Fuji Photo Film Co., Ltd., Odawara-shi, Kanagawa (JP); Uchiyama, Kimiyoshi, c/o Fuji Photo Film Co., Ltd., Odawara-shi, Kanagawa (JP); Sato, Kaoru, c/o Fuji Photo Film Co., Ltd., Odawara-shi, Kanagawa (JP)
(74) Representative: Grünecker, Kinkeldey, Stockmair & Schwanhäusser Anwaltssozietät

(57) **Abstract**

Disclosed is a method of wrapping photographic treating agents with a wrapping composite lamination material of two or more materials not containing Al and/or Cl. Such wrapping materials when burnt for disposal can cause no damage on furnaces.

## Description

### Background of the Invention:

### Field of the Invention:

The present invention relates to a method of wrapping photographic treating agents.

### Description of the Prior Art:

After being exposed to light, monochrome photosensitive films are subjected to developing, fixing and rinsing. Likewise, after being exposed to light, color photosensitive films are subjected to color-developing, silver-removing, rinsing, stabilizing and so forth. Different liquids are used such as monochrome or color-producing developing liquid, fixing liquid, bleach liquid for removing silver, bleach fixing liquid, tap water or ion exchange water for rinsing, and stabilizing liquid. Usually, these liquids are heated at the temperature ranging from 20 to 50 °C, and photosensitive films are put in the bath of such a treatment liquid. These liquids are prepared from different photographic treating agents, most of which are in solid state.

Such photographic treating liquids may be prepared by customers. For the sake of convenience, however, photographic treating liquids are thickened for sale. Then, customers dilute such concentrates before using. Transportation of photographic treating agents in liquid phase, however, causes many problems. Photographic treating agents in solid state for instance, pulverized treating agents are convenient to transportation. Recently in view of this and other factors solid photographic treating agents have been thought better of.

As a matter of fact solid chemicals must be used in preparing photographic treating agents, and usually these solid chemicals are stored until their use.

Among such photographic treating agents some chemicals are liable to change if they are exposed to water or oxygen, and certain chemicals when pulverized and mixed, come to be unstable in the presence of water or oxygen. In this connection there is an anxiety for deterioration of photographic treating agents for an elongated period of preservation. Examples of such chemicals are hydroquinone, alkalis and reducing agents.

In the hope of preventing deterioration such chemicals which are liable to deteriorate in preservation are wrapped by resin-coated or vinylidene chloride-coated aluminum foil, which provides an oxygen-and-water barrier.

After being used these wrapping materials are burnt for disposal, and then, these materials containing Al or Cl are likely to damage furnaces. Therefore, there has been a demand for wrapping materials the burning of which causes no damage on furnaces.

### Summary of the Invention:

One object of the present invention is to provide a wrapping material not containing Al and/or Cl and being capable of preventing deterioration of photographic chemicals for an elongated period of preservation.

To attain this object a method of wrapping photographic treatments according to the present invention comprises the steps of: preparing a wrapping composite lamination material of two or more materials not containing Al and/or Cl, the oxygen permeability of which composite lamination material is below 10 ml/m²atm at 25 °C for 24 hours, and the water permeability of which composite lamination material is below 5 ml/m²atm at 25°C for 24 hours, and wrapping photographic treating agents of solid state by said composite lamination material.

According to one aspect of the present invention said wrapping composite lamination material contains at least one of extensible polypropylene, polyethylene vinyl alcohol and siliconoxide; and a heat-sealing material is laid on said wrapping composite lamination material.

According to another aspect of the present invention wrapping is effected by preparing a wrapping bag from said wrapping composite lamination material and putting solid photographic agents in said bag, preparation of said bag begining with its bottom, followed by putting said photographic treating agents in the bag, and ending with sealing the opening top of the bag.

According to still another aspect of the present invention photographic treating agents of solid state are wrapped doubly by using a double bag, each of its inner and outer bags being of materials not containing Al and/or Cl.

Other objects and advantages of the present invention will be understood from the following description of preferred embodiments of the present invention with reference to accompanying drawings:

Figs. 1a, 1b and 1c show schematically the manner in which a gusseted bag is prepared.

Solid photographic chemicals are wrapped by a wrapping composite lamination material of two or more materials not containing Al and/or Cl. The oxygen permeability of the wrapping composite lamination material is below 10 ml/m²atm at 25 °C for 24 hours, preferably below 5 ml/m²atm at 25°C for 24 hours, and the water permeability of the wrapping composite lamination material is below 5 ml/m²atm at 25°C for 24 hours, preferably below 2 ml/m²atm at 25 °C for 24 hours. As a matter of fact the oxygen permiability and water permeability of the wrapping material, the smaller, the better, can be reduced to about 0.1 ml/m²atm at 25°C for 24 hours.

Such composite laminations can prevent invasion of oxygen and water into the wrapping, thus preventing deterioration of photographic chemicals for an elongated storage.

A conventional wrapping material which is capable of preventing invasion of water or oxygen such as resin-coated aluminum foil or polyvinylidene fluoride-lined sheet, however, contains Al or Cl, and therefore, it is likely that such a wrapping material when burnt for disposal damages the furnace. In other words, a wrapping material containing neither Al nor Cl cannot damage the furnace.

The oxygen permiability of the wrapping material in the form of sheet or film was determined according to the Mocor method whereas the water-permeability of the wrapping material in the form of sheet or film was determined according to the Cup method.

Examples of the material which is capable of preventing invasion of water are oriented polypropylene (OPP), silicon dioxide etc. Examples of the material which is capable of preventing invasion of oxygen are polyethylene vinyl alcohol (EVAL), silicon dioxide, polyethylene terephthalate (PET) etc.

Polyethylene vinyl alcohol may be partly saponified.

Some materials selected among these are used in combination to provide a lamination. It is important that the material which comes to contact photographic chemicals to be wrapped causes no adverse effect on such photographic chemicals. Two or more layers of one and same material can be laid on each other.

OPP, EVAL, PET or other resin materials may be in the form of film, and these films may be laid on each other to provide a composite lamination according to a well known method.

Silicon dioxide coating may be formed on composite laminations according to the chemical or physical vapor phase growing method. Preferably, such coating may be formed by vapor deposition or sputtering. Silicon dioxide coating may be in the form of SiOₓ, the coating thickness depending on a particular coating method taken. It may be formed by applying SiO₂ on a substrate when occasions demand.

One resin layer in a composite lamination is 5 to 100 µ m thick, preferably 10 to 50µ m thick. An SiO₂ coating is 0.4 to 0.8µ m thick. The composite lamination is 20 to 120 µ m thick, preferably 30 to 60µ m thick.

If a composite lamination contains at least one of OPP, EVAL and SiO₂ layers, the lamination preferably contains a heat-sealing layer.

Examples of such heat-sealing materials are polyethlene (PE), linear low-density polyethylene (LLDPE), PET, polypropylene (PP) and other resin materials.

Addition of such heat-sealing layer improves the flexibility of the composite lamination, and provides a crease-free wrapping material.

A heat-sealing layer is 20 to 150 µ m thick, preferably 30 to 80 µ m thick. A composite lamination having such a heat-sealing layer is 40 to 200 µ m thick, preferably 50 to 120µ m thick.

Some examples of wrapping material according to the present invention are:

### (1) (outside) OPP/EVAL/PE (photographic chemicals)

OPP film is 10 to 30µ m thick; EVAL film is 10 to 30 µ m thick; and PE is 40 to 80 µ m thick. The oxygen permeability of the composite lamination is 0.2 to 1.5 ml/m²atm at 25°C for 24 hours, and the water permeability of the composite lamination is 3.5 to 5.0 ml/m²atm at 25°C for 24 hours.

### (2) (outside) PET/SiO₂/PET/LLDPE (photographic chemicals)

PET film is 10 to 20µ m thick; SiO₂ coating is 0.4 to 0.8µ m thick; PET film is 10 to 20 µ m thick; and LLDPE is 40 to 80 µ m thick. The oxygen permeability of the composite lamination is 0.1 to 1.0 ml/m²atm at 25 °C for 24 hours, and the water permeability of the composite lamination is 0.1 to 1.0 ml/m²atm at 25 °C for 24 hours.

Preferably a wrapping material according to the present invention may be used in the form of gusseted bag.

Figs. 1a, 1b and 1c show schematically sequential steps of preparing a gusseted bag of a wrapping material according to the present invention.

As shown in Fig. 1a, a bottomless bag 1 is prepared, and then its bottom is closed to form the flat bottom 10 of the bag 1. Then, as shown in Fig. 1b, photographic chemicals 2 are put in the bag 1. Finally, as shown in Fig. 1c, the top of the bag 1 is closed and sealed. Thus, a gusseted enclosure 15 results. Use of a lamination having a sheet of heat-sealing-material therein is effective to cause no creases on the bottom 10 of the gusseted bag.

The size of gusseted bags may be determined to be appropriate for the purpose. Usually the bag capacity is 200 to 10,000 ml.

Such gusseted bags can be laid on each other to form a stack, which is convenient to storage.

In place of forming gusseted bags from a composite lamination double gusseted bags may be formed, each having inside and outside bags of wrapping materials not containing Al and/or Cl to wrap photographic chemicals doubly.

Specifically the inside bag to contain photographic chemicals may be made of materials which have no adverse effect on the content, such as PE, PET, PP or other resin materials. It may be of a single layer of a material guaranteed free of ill effects, or of a composite lamination of such a single layer and a nylon film.

Preferably, the space between the inner and outer bags of a double gusseted bag may be filled with a gas which causes no effect on the photographic chemicals inside.

The oxygen permeability of the outside enclosure of such a double gusseted bag is below 20 ml/m²atm at 25 °C for 24 hours, preferably below 10 ml/m²atm at 25°C for 24 hours, and the water permeability is below 10 ml/m²atm at 25 °C for 24 hours, preferably below 5 ml/m²atm at 25 °C for 24 hours. More preferably, the oxygen and water permeability of the outside enclosure may be below 5 ml/m²atm at 25 °C for 24 hours.

Examples of materials whose oxygen permeability is around the prescribed value are nylon, PET, EVAL and other resin materials whereas examples of materials whose water permeability is around the prescribed value are OPP, PET and other resin materials. Preferably, two or more materials are selected among these materials to form a composite lamination.

Double gusseted bags are equally effective to prevent deterioration of photographic chemicals inside, and such bags cause no trouble when burnt for disposal.

The outer enclosure of such a double gusseted bag may be 20 to 150µ m thick, preferably 30 to 60µ m thick, where as the inside enclosure may be 30 to 150µ m thick, preferably 40 to 80 µ m thick.

The space between the inner and outer bags of a double gusseted bag may be filled with N₂ or any other gas appropriate for the purpose, which filler gas are selected among those which cause no problems for disposal. Such space may be filled with a desiccating agent such as silica gel.

Different photographic chemicals which are used in preparing monochrome or color-producing developing liquid, fixing liquid, bleach liquid for removing silver, bleach fixing liquid or stabilizing liquid can be wrapped according to the wrapping method of the present invention.

The wrapping is appropriate for the purpose of preserving for an elongated period such photographic chemicals which are liable to deteriorate by oxidization and moisture absorption.

Examples of such chemicals are a dihydroxybenzene such as hydroquinone, a pyrazolidone such as pyrazone and other developing agents, thiosulfate and other fixing agents, a sulfite such as Na₂S₂O₅ or NaSO₃, and an alkali agent such as NaOH, KOH or K₂CO₃.

In case that some pulverized treating chemicals are combined, these chemicals in combination are liable to absorb water easily or liable to be oxidized easily. Examples of trouble-free treating agent combinations are: developing agents and alkalis; sulfites and acid agents; and thio sulfates and acid agents.

The compositions of some examples of treating liquids prepared by using selected photographic treating agents and the conditions in which such treating liquids are prepared are described in detail in Japanese Patent Application Public Disclosure Nos. 2-103035; 2-103037; 2-71260; and 61-267559 (monochrome photosensitive material), and in Japanese Patent Application Public Disclosure Nos. 63-70857; and 1-190889 (color photosensitive material).

The present invention is described in terms of some selected examples as follows:

### EXAMPLE 1

| The composition of a monochrome developing liquid is: | |
|---|---|
| sodium hydroxide (NaOH): | 40g |
| borax: | 15g |
| potassium bromide (KBr): | 2g |
| 1-phenyl-5-mercaptoterazole: | 0.05g |
| sodium sulfite: | 60g |
| hydroquinone: | 30g |
| 1-phenyl-3-pyrazolidone: | 3g |
| ethylenediamine tetra acetic acid (EDTA): | 1.0g |
| water added: | 1 liter |

These ingredients excluding water are solid.

These ingredients are separated in groups each made up by: NaOH and borax; sodium sulfite, KBr and EDTA; and hydroquinone, 1-phenyl-5-mercaptoterazole, and 1-phenyl-3-pyrazolidone. Then, gusseted bags (1000 ml) were prepared and filled with such grouped photographic chemicals, identified as Treating Agent A. The gusseted bag lamination is: OPP(20 µ m thick)/EVAL(15µ m thick)/PE(50µ m thick). The oxygen permeability of the lamination is 0.5 ml/m²atm at 25°C for 24 hours, and the water permeability is 4 ml/m²atm at 25°C for 24 hours. The chemical content is on the side of PE.

Treating Agent A were stored at 50°C, 90% RH for one month, and then, monochrome developing liquid A was prepared from the treating agent.

Minicopy microfilm HR-11, monochrome photographic film produced by FUJI PHOTO FILM Co., LTD was exposed to light. Then, it was subjected to monochrome development (20 seconds; 38 °C ); fixing (20 seconds; 25 °C ); rinsing (20 seconds; 25 °C ); and drying (40 seconds; 65 °C).

Monochrome developing liquid A was used, and a fixing liquid used had the following composition:

| | |
|---|---|
| ammonium thio sulfate: | 120g |
| sodium thio sulfate: | 30g |
| sodium sulfite: | 10g |
| boric acid: | 8g |
| tataric acid: | 1.0g |
| aluminum sulfate: | 15g |
| potassium iodide: | 0.05g |
| water added: | 1 liter |

Minicopy microfilm HR-11 was exposed to light. Then, it was subjected to monochrome development using the standard monochrome developing liquid having same composition as monochrome developing liquid A, and was subjected to sequential treatments as described above.

The development characteristics (sensitivities, fogging etc.) of the exposed film treated with monochrome developing liquid A were found to be as good as those of the one treated with the standard monochrome developing liquid.

### EXAMPLE 2

The same solid ingredients as the fixing liquid in EXAMPLE 1 are separated in two groups each made up by: ammonium thio sulfate, sodium thio sulfate, and sodium sulfite; and boric acid, tataric acid and aluminum sulfate. Then, gusseted bags were prepared for each group, and were identified as Treating Agent a. The gusseted bag composition is the same as in EXAMPLE 1.

Treating Agent a was stored in the same condition in EXAMPLE 1, and a fixing liquid a was prepared from the treating agent.

A standard fixing liquid was prepared from same ingredients which had not been stored.

Photographic films were exposed to light and subjected to monochrome developing with the standard developing liquid, fixing and sequential treatments.

No poor fixing areas were detected in the films which were treated with the fixing liquid a, as was the case with the ones which were treated with the standard fixing liquid.

Also, in EXAMPLES 1 and 2 another gusseted bags each composed of PET (12 µ m thick)/SiO₂ (0.5µ m thick)/ PET (12 µ m thick)/LLDPE (50µ m thick) were used to store developing and fixing ingredients for same period, and then, the developing and fixing liquids were prepared. Same experiments were made only to find that: these photographic treating agents had as good characteristics as those packed in the first gusseted bags above described and stored and similar good results were obtained.

The oxygen permeability of the composite lamination thus used was 0.5 ml/m²atm at 25°C for 24 hours, and the water permeability was 0.5 ml/m²atm at 25 °C for 24 hours.

In addition, in EXAMPLES 1 and 2 double-gusseted bags were used, each comprising an 80µ m -thick inner bag of PET and an outer bag, the lamination film of which outer bag was composed of OPP (20 µ m thick)/nylon (15µ m thick)/PET (25 µ m thick), the oxygen and water permeabilities of the lamination film being 10 and 5 ml/m²atm at 25 °C for 24 hours. The space between the outer and inner bags of each double gusseted bag is filled with N₂.

These double-gusset bags were used to store developing and fixing chemicals for same period, and then, the developing and fixing liquids were prepared. Same experiments were made only to find that these photographic treating agents had as good characteristics as those which were packed in the gusset bags above described and stored, and similar good results were obtained.

All wrapping materials contain neither Al nor Cl, and therefore, the gusseted bags when burnt caused no damage on the furnace.

As is apparent from the above, anti-oxidizing and anti-hygroscopic wrapping materials used in the wrapping method according to the present invention contain neither Al nor Cl, and therefore, such materials when burnt for disposal can cause no damage on the furnace.

## Claims

1. Method of wrapping photographic treating agents characterized in that it comprises the steps of: preparing a wrapping composite lamination material of two or more materials not containing Al and/or Cl, the oxygen permeability of which composite lamination material is below 10 ml/m²atm at 25 °C for 24 hours, and the water permeability of which composite layer material is below 5 ml/m²atm at 25°C for 24 hours, and wrapping photographic treating agents of solid state by said wrapping composite lamination.

2. Method of wrapping photographic treating agents according to claim 1 wherein said wrapping composite lamination material contains at least one of extensible polypropylene, polyethylene vinyl alcohol and siliconoxide, and a heat-sealing material is laminated on said wrapping composite lamination material.

3. Method of wrapping photographic treating agents according to claim 1 or 2 wherein wrapping is effected by preparing a wrapping bag from said wrapping composite lamination material and putting said photographic treating agents in said bag, preparation of said bag begining with its bottom, followed by putting said photographic treating agents in the bag, and ending with sealing the opening top of the bag.

4. Method of wrapping photographic treating agents characterized in that it comprises the step of wrapping doubly photographic treating agents of solid state by using a double bag of materials not containing Al and/or Cl.
